

## UNITED STATES PATENT OFFICE

2,523,324

## TANNING WITH ESTERS OF CHLOROFORMIC ACID IN A NONAQUEOUS MEDIUM

Robert C. Putnam, Marblehead, Mass., assignor  
to United Shoe Machinery Corporation, Flemington, N. J., a corporation of New Jersey

No Drawing. Application April 23, 1947, Serial  
No. 743,459

5 Claims. (Cl. 8—94.33)

1

My invention relates to the treatment of hides and skins.

In the well-known chrome tanning process, a skin or hide pretreated to remove hair and treated by various other steps such as bating and pickling, is immersed for an extended period in a solution of basic chromium sulphate. Ordinarily this chromium treatment of the skin or hide is carried on in a "paddle" or a drum during the chrome treating period and is then removed from the "paddle" or drum and aged for a period of from several hours up to two days.

In the vegetable tanning process, dehaired and otherwise pretreated skins or hides are subjected to various steps including a prolonged soaking treatment in a solution containing various vegetable extracts. Tanning by the vegetable method occupies a period of several weeks and involves extensive handling of the hides.

By either of these common methods of tanning, extended periods of time are required so that to insure continuous production of leather a very large number of skins or hides must be maintained in various stages of tanning. Investment in skins or hides and in treating tanks, vats, or other treating equipment is large so that the cost of the ultimate leather is high.

It is an important feature of my invention to convert skin and hide material to a stable non-putrescible leather-like condition by a short and simple treatment of the skin or hide materials with a new type of reagent. By my new process there is formed a tough, pliable product similar to leather in appearance and in many other properties. The new product will withstand prolonged soaking in water without marked shriveling or hardening even at relatively high temperatures, and is exceptionally resistant to mold growth.

I have discovered that skins or hides may be converted to this novel leather-like material by drying the skin or hide material and contacting the dried material with chloroformates. These chloroformates are ordinarily employed in the form of solutions which readily penetrate the skin or hide. I have made the further discovery that a product possessing increased softness and flexibility and an improved appearance is formed where certain special solvents are employed in combination with the active treating agents.

For treatment according to the process of the present invention, I have found that bated or pickled and hairy skins or hides, for example calfskins or steer hides, are very satisfactory. Skins or hides in other conditions, such as de-limed skins or hides, may also be used. For most

2

satisfactory treatment, the hide or skin should have a pH of between about 5 and about 7 prior to treatment. However, skins or hides having a pH somewhat outside these approximate limits may be treated.

Skins or hides of animals generally used for making leather may be treated according to the process of the present invention. In the specification and claims the terms "skin" or "skin material" are to be understood in their broad sense as including these materials. The term "tanning" as employed in the claims is to be understood as covering the process of reacting the treating agents of the present invention with skins or hides to form a leather-like material and is not to be understood as requiring the action of tannic acid or tannins.

Where a pickled material is used, it is first subjected to a conventional depickling operation.

20 The depickled skin is then immersed in water with agitation to remove dissolved salts and other soluble materials. A suitable treatment period may range from around 2 hours for calf-skin to 4 hours for a steer skin.

25 The depickled and soaked skin is then dried to a moisture content which may be between about 10 and about 15%. This moisture content is determined by comparison with the weight of the skin when subjected to a further drying for 16 hours in air at 105° C. It has been found that drying is most satisfactorily accomplished by the action of solvents, for example, acetone, methyl acetate, isopropyl alcohol, dioxane, ethylene glycol monomethyl ether acetate or other solvent which will remove the water without seriously harming the skin. This drying may be effected by leaving the skin immersed in an agitated bath of the solvent overnight. The solvent is then removed from the skin, suitably by evaporation in a stream of dry warm air.

30 The above is but one of many conceivable methods for treatment of a skin prior to the treatment with my new agents. Modifications will be readily apparent to persons familiar with the handling of skins. For example, a bated skin need not be subject to the depickling and washing operations above outlined.

35 The dried skin is immersed in a body of the liquid treating agent and is maintained in the liquid for a sufficient period to convert the skin to the new leather-like condition.

40 I have found that the bis-chloroformates of glycols, polyglycols and sulfur-substituted glycols and polyglycols are very effective treating agents. Among compounds in this class are glycol bis-

chloroformate, di, tri, tetra and dodeca-ethylene glycol bis-chloroformates, tri-methylene glycol bis-chloroformate, and mercapto-ethanol bis-chloroformate.

Other chloroformates which have been found satisfactory include chloroformates of aliphatic hydrocarbons such as methyl chloroformate, ethyl chloroformate, butyl chloroformate, iso-butyl chloroformate, amyl chloroformate, hexyl chloroformate, lauryl chloroformate and stearyl chloroformate, the aromatic chloroformates such as phenyl chloroformate and benzyl chloroformate, and  $\beta$  chloro ethyl chloroformate.

I have made the further surprising discovery that skins are converted to a leather-like material having particularly good resistance to deterioration under the action of water by treating them with chloroformates of higher aliphatic hydrocarbons such as lauryl and stearyl chloroformates having up to 18 carbon atoms.

These treating agents are ordinarily employed as organic solvent solutions in order that they may penetrate well into the interior of the skin material, and in order to avoid a too vigorous reaction between the material and the treating agent. Diethylene glycol monomethyl ether formal has been found particularly satisfactory as a solvent for the treating agent, and solutions comprising it convert skin to particularly soft and fine-appearing, leather-like products. Ethylene glycol monomethyl ether formal and tri-chlorethylene have been used as solvents with many of applicant's treating agents, and the solutions have been found to give very desirable products. Other organic solvents, such as acetone, hexane, carbon tetrachloride, butyl carbitol formal, the diethylene glycol monomethyl ether tetra acetal of glyoxal or toluene, for the agents may be used. A preferred range of concentrations of solutions is from about 10% to about 50% treating agent by volume based on the volume of the solution.

The time of immersion of the skin in the treating agent varies with the weight and type of skin treated. Preferred times of treatment may vary from about one-half hour to about five hours. In the case of a calfskin, satisfactory action has been obtained by immersion of the prepared, dried, calfskin for about two hours at 130° F. in a fifty per cent solution of di-glycol bis-chloroformate in diethylene glycol monomethyl ether formal. In the case of steer hide, a four hour immersion in the same solution at 130° F. has been found satisfactory.

Comparable effects on these materials have been obtained within the same treating time using as treating agent a fifty per cent solution of di-glycol bis-chloroformate in tri-chlorethylene at room temperature.

As illustrated above, the temperature of the treating bath may vary. Factors controlling the temperature include the boiling points and vapor pressure of the solvents and of the treating agents and the rate of treating action desired.

After the above treatment, the skin is removed from the treating bath and is immersed in a solvent to remove soluble materials such as excess agent, reaction products and the like. Suitable solvents for this use are trichlorethylene, acetone and toluene.

The skin is removed from the solvent bath and is permitted to dry. The dried skin is then placed in a neutralizing bath, which may be a depickling solution, until it reaches a pH of about 7 or other value depending upon the properties

desired. This step is desirable in that it also serves to neutralize or decompose acid compounds which may have formed within the skin. The skin is finally washed to remove salts, and is then removed from the washing bath.

The treated skin may be subjected to such further treatments as desired, for example, dyeing, fat liquoring or stuffing, drying and surface finishing.

10 The following examples are given as illustrative of processes in accordance with the present invention. It is to be understood that the invention is not restricted to the reagents and procedural details disclosed in these examples.

15 Example 1.—A steer hide (butt) in the bated condition was immersed overnight in acetone to dry the hide. The hide was removed from the acetone and was subjected to a blast of warm air to evaporate the acetone. The resulting hide 20 had a moisture content of about 10 per cent determined by the method noted above. The dried hide was then immersed in a treating bath at room temperature, the treating bath consisting of 20 parts by volume of di-glycol chloroformate 25 and 80 parts by volume of tri-chlorethylene. After five hours the hide was removed and washed for two hours in a bath consisting only of tri-chlorethylene. After washing, the hide was removed and allowed to dry and was then 30 immersed in a bath of 5 per cent sodium bicarbonate in water until the hide reached a pH of about 7. The neutralized hide was removed from the bicarbonate solution and placed in a bath of running water for two hours. The neutralized and washed hide was removed and found 35 to be in a leather-like condition in which it could be subjected to operations following conventional tanning.

Example 2.—Pickled calfskin was depickled by 40 immersion in a 5 per cent aqueous solution of sodium bicarbonate for an hour. The depickled skin was washed in running water for an hour and dried overnight in a bath of acetone. The calfskin was removed from the acetone and the 45 acetone evaporated from the calfskin by a blast of warm air. The dried skin was then immersed for two hours in a treating bath at a temperature of 130° F., the treating bath consisting of 50 parts by volume of tri-ethylene glycol bis-chloroformate and 50 parts by volume of diethylene glycol monomethyl ether formal. The treated calfskin was removed from the bath and washed for two hours in acetone after which it was removed and allowed to dry. The dried calfskin 55 was then immersed in a 5 per cent solution of sodium bicarbonate until substantially neutral and was then washed for two hours in running water. The calfskin was removed from the water and found to be in a stable non-putrescible condition 60 in which it could be subjected to the usual operations which follow tanning.

Example 3.—A calfskin in bated condition was dried overnight in acetone and was removed from the acetone and subjected to a blast of warm air 65 to evaporate the acetone. The dried calfskin was then immersed in a bath consisting of 50 parts by volume of lauryl chloroformate and 50 parts by volume of tri-chlorethylene for two hours at room temperature. The treated material was 70 then washed for two hours in trichlorethylene, removed and allowed to dry. The dried calfskin was then neutralized to a pH of about 7 in a 5 per cent solution of sodium bicarbonate. The neutralized skin was finally washed for two hours 75 in running water and gave a leather-like mate-

rial in condition for the usual operations following tanning.

Having described my invention, what I claim as new and desire to secure by Letters Patent of the United States is:

1. The method of tanning stock having a moisture content of from 10% to 15% which comprises contacting the stock with an organic solvent solution of an ester of chloroformic acid in an organic solvent, the concentration of the solution being from about 10% to about 50% of the ester of chloroformic acid based upon the volume of the solution.

2. The method of tanning stock which comprises drying the stock by the solvent action of an organic liquid to bring the moisture content down to from about 10 per cent to about 15 per cent and contacting the dried stock with an organic solvent solution of at least one member of the group consisting of bis-chloroformates of glycols and polyglycols, chloroformates of alkyl hydrocarbons having up to 18 carbon atoms, phenyl and benzyl chloroformates, mercaptoethanol bis-chloroformate and  $\beta$  chloroethyl chloroformate, the concentration of the solution being from about 10 per cent to about 50 per cent of treating agent based upon the volume of the solution.

3. The method of tanning stock which comprises drying the stock by the solvent action of an organic liquid to bring the moisture content down to from about 10 per cent to about 15 per cent, contacting the dried stock with a solution of di-glycol bis-chloroformate in diethylene glycol monomethyl ether formal, the concentration of di-glycol bis-chloroformate in the solution being from about 10 per cent to about 50 per cent by volume based upon the volume of the solution, maintaining the stock in contact with the solution for a period corresponding to from about two hours for a calfskin to about four hours for a steer-hide at a temperature of 130° F., removing uncombined di-glycol bis-chloroformate by the action of a solvent, neutralizing acid compounds which may have formed within the stock, washing the stock to remove neutral salts, and drying the stock.

4. The method of tanning stock which comprises drying the stock by the solvent action of an organic liquid to bring the moisture content down to from about 10 per cent to about 15 per cent, contacting the dried stock with a solution of benzyl chloroformate in diethylene glycol monomethyl ether formal, the concentration of benzyl chloroformate in the solution being from

about 10 per cent to about 50 per cent by volume based upon the weight of the solution, maintaining the stock in contact with the solution for a period corresponding to from about two hours for a calfskin to about four hours for a steer hide at a temperature of 130° F., removing uncombined benzyl chloroformate by the action of a solvent, neutralizing acid compounds which may have formed within the stock, washing the stock to remove neutral salts, and drying the stock.

5. The method of tanning stock which comprises drying the stock by the solvent action of an organic liquid to bring the moisture content down to from about 10 per cent to about 15 per cent, contacting the dried stock with a solution of lauryl chloroformate in diethylene glycol monomethyl ether formal, the concentration of lauryl chloroformate in the solution being from about 10 per cent to about 50 per cent by volume based upon the weight of the solution, maintaining the stock in contact with the solution for a period corresponding to from about two hours for a calfskin to about four hours for a steer hide at a temperature of 130° F., removing uncombined lauryl chloroformate by the action of a solvent, neutralizing acid compounds which may have formed within the stock, washing the stock to remove neutral salts, and drying the stock.

ROBERT C. PUTNAM.

30

#### REFERENCES CITED

The following references are of record in the file of this patent:

#### UNITED STATES PATENTS

|    | Number    | Name       | Date          |
|----|-----------|------------|---------------|
| 35 | 501,235   | Seifert    | July 11, 1893 |
|    | 1,789,322 | Roark      | Jan. 20, 1931 |
|    | 1,826,690 | Carroll    | Oct. 6, 1931  |
| 40 | 2,080,019 | White      | May 11, 1937  |
|    | 2,127,841 | Gellendien | Aug. 23, 1938 |
|    | 2,169,513 | Brunkens   | Aug. 15, 1939 |
|    | 2,186,889 | Ulrich     | Jan. 9, 1940  |

#### FOREIGN PATENTS

|    | Number  | Country       | Date          |
|----|---------|---------------|---------------|
| 45 | 461,179 | Great Britain | 1937          |
|    | 509,703 | Great Britain | July 19, 1939 |
|    | 447,715 | Belgium       | Oct. 27, 1942 |
| 50 | 118,155 | Australia     | Jan. 9, 1943  |

#### OTHER REFERENCES

"Richter's Organic Chemistry" by Spielman, vol. I, pub. 1919 by P. Blakiston's Son and Co., Phila., Pa., page 430.

55